# EUROPEAN PATENT SPECIFICATION

(11) **EP 1 026 273 B1**
(45) Date of publication and mention of the grant of the patent: **19.12.2007**
(21) Application number: 98932588.1
(22) Date of filing: 17.07.1998
(51) Int. Cl.: C22C 38/00, C22C 38/40, C22C 38/42, C22C 38/50

(54) **MARTENSITE STAINLESS STEEL OF HIGH CORROSION RESISTANCE**
MARTENSITISCHER ROSTFREIER STAHL MIT HOHEM KORROSIONSWIDERSTAND
ACIER INOXYDABLE MARTENSITIQUE A HAUTE RESISTANCE A LA CORROSION

(30) Priority: 18.07.1997 JP 19400097
(43) Date of publication of application: 09.08.2000
(73) Proprietor: Sumitomo Metal Industries Limited, Osaka-shi, Osaka 541-0041 (JP)
(72) Inventor: UEDA, Masakatsu, Sumitomo Metal Ind., Ltd., Wakayama-shi, Wakayama 640-8555 (JP); TAKABE, Hideki, Sumitomo Metal Ind., Ltd., Wakayama-shi, Wakayama 640-8555 (JP); KONDO, Kunio, Sumitomo Metal Ind., Ltd., Osaka-shi, Osaka 541-0041 (JP); OGAWA, Kazuhiro, Sumitomo Metal Ind., Ltd., Osaka-shi, Osaka 541-0041 (JP); AMAYA, Hisashi, Sumitomo Metal Ind., Ltd., Osaka-shi, Osaka 541-0041 (JP)
(74) Representative: Uchida, Kenji
(86) International application number: PCT/JP1998/003243
(87) International publication number: WO 1999/004052

(56) References cited:
- EP-A- 0 273 279
- JP-A- 4 268 019
- JP-A- 6 299 301
- JP-A- 8 041 599
- JP-A- 8 199 236
- PATENT ABSTRACTS OF JAPAN vol. 018, no. 430 (C-1236), 11 August 1994 (1994-08-11) & JP 06 128632 A (NIPPON STEEL CORP), 10 May 1994 (1994-05-10)

## Description

### Technical Field

This invention relates to a high-corrosion-resistant martensitic stainless steel for use under cathodic protection. This stainless steel has excellent corrosion resistance in atmospheres, which contain carbon dioxide, and, therefore, it is suitable for use in line-pipes for transporting oil and natural gas, which contain carbon dioxide. Even if the pipe is used in a welded condition in the sea with cathodic protection, there is no risk that the pipe will suffer cracking.

The stainless steel of this invention is preferably used as a material for seamless pipes, resistance welded pipes, laser welded pipes, submerged arc welded (SAW) pipes and the like. In steel products other than pipes, such as plates, bars, and shape steels, this stainless steel may also be used as a material for various types of equipment exposed to atmospheres, which contain carbon dioxide. Such equipment includes, e.g., piping for decarbonating facilities, piping for geothermal power generation, and tanks for carbon dioxide-containing liquids. Furthermore, the stainless steel according to this invention can be used in environments, which contain a slight amount of hydrogen sulfide together with carbon dioxide.

### Background Art

Recently, the environments in wells for collecting oil or natural gas have become increasingly severe, and thus the corrosion of pipes for transporting these fluids has become a serious problem.

In order to prevent this corrosion problem, the following measures have conventionally been taken.
(1) When carbon steels are used as piping materials, inhibitors for preventing corrosion are used.
(2) Duplex stainless steels, having excellent corrosion resistance, are used as piping materials.

In either case, pipes to be laid down in the seawater are subjected to a cathodic protection process in order to protect the outer surfaces from corrosion.

In the method described in the first method (1) above, the pipes themselves are inexpensive, but the inhibitors are expensive and could cause environmental pollution. On the other hand, the duplex stainless steels in the second method (2) are expensive.

Many research papers are available on the corrosion resisting performance of a steel against carbon dioxide (hereinafter referred to as "corrosion resistance to carbon dioxide"). For example, it is reported by A. Ikeda et al., in Corrosion/83, NACE Houston. Paper No. 45, 1983, that a steel containing 7% or more Cr can be protected from carbon dioxide corrosion in an aqueous solution, which is as high as about 100°C and contains carbon dioxide. Further, M. Ueda et al. disclose in Corrosion/92, NACE Houston. Paper No. 55, 1992, that the localized corrosion resistance of a 13Cr martensitic stainless steel is improved by adding Mo and/or W.

On the basis of the above-described research results, attention has been paid recently to a 13Cr martensitic stainless steel, e.g., JIS SUS 410 steel, as a piping material which is resistant to carbon dioxide corrosion. A steel of this grade is used after subjected it to a quenching-tempering heat treatment. When welded, the steel is subjected to a post weld heat treatment (hereinafter abbreviated as "PWHT"), for the purpose of assuring the toughness at welds and preventing delayed fracture (Kenji Satoh et al.: Corrosion/83, NACE Houston, Paper NO. 56, 1983).

Martensitic stainless steels are comparatively inexpensive, exhibit high strength and excellent corrosion resistance, and can be used without inhibitors. However, when used, e.g., as an undersea pipeline or the like in the seawater, the martensitic stainless steel needs to be subjected to cathodic protection for the prevention of corrosion to the outer surface, and when subjected to the cathodic protection, there arises a serious problem which is never encountered by carbon steels and duplex stainless steels.

Cathodic protection is a corrosion prevention method in which the corrosion current is cancelled by producing a protective current using a steel material to be corroded as the cathode. During this process, hydrogen is produced by the cathodic reaction, and the produced hydrogen is absorbed into the steel material. The welding heat affected zone of a 13Cr martensitic stainless steel has a quenched structure as welded, and exhibits an extreme hardness. When hydrogen is absorbed into such a zone, it suffers cracking due to hydrogen embrittlement.

It is thought that the cracking due to cathodic protection can be prevented to some degree by a heat treatment after welding (PWHT). However, for the conventional 13Cr martensitic stainless steel, the PWHT is not sufficient to reliably prevent the cracking caused by cathodic protection. In addition, it is comparatively easy to carry out the PWHT at a pipe making plant, but a PWHT, which is to be carried out after a peripheral welding at a site during the laying down of a pipeline, leads to a large increase in the operational costs.

From the above-described circumstances, there has been a strong demand for a martensitic stainless steel, free from the previously described cracking accompanied by cathodic protection. However, no martensitic stainless steel intended to prevent the cracking at the welding heat affected zone, due to cathodic protection, has yet been proposed. U.S. Patent No. 5,383,983 (corresponding to Japanese Unexamined Patent Application Laid-Open No. 5-287455(1993)) discloses a martensitic stainless steel, which contains Ti or Zr as essential elements in the chemical composition and exhibits an excellent corrosion resistance. However, no consideration is given to that steel for the prevention of the cracking due to cathodic protection.

### Disclosure of the Invention

One of the objects of this invention is to provide a martensitic stainless steel having all of the following properties (a) to (c).
(a) To have an excellent corrosion resistance, particularly, in environments which contain carbon dioxide or a slight amount of hydrogen sulfide together with carbon dioxide.
(b) To have a proof stress (0.2% proof stress) of 550MPa (80ksi) or more when quenched and tempered.
(c) To have no risk of cracking due to cathodic protection, even if used as welded without a PWHT.

Another object of this invention is to provide a steel pipe, which is made of a martensitic stainless steel, having the above-described properties as a material. This steel pipe includes seamless pipes, and welded pipes such as resistance welded pipes, laser welded pipes, and SAW pipes.

The basic chemical composition of the martensitic stainless steel according to this invention is as follows.

The basic composition consists on a mass basis, of: C: not greater than 0.04%, Si: 0.01-1.0%, Mn: 0.1-1.5%, Cr: 7-15%, Ni: 0.7-less than 4.0, Al: 0.001-0.20%, Cu: 0-2%, S: not greater than 0.01%, N: not greater than 0.05%, and a balance of Fe and incidental impurities.

In addition, the composition may further contain one or more of alloying elements selected from at least one of the following first group elements, second group elements, and third group elements:
- First group elements: Nb: 0.005-0.10%, Ti: 0.005-0.10%, and Zr: 0.005-0.10%;
- Second group elements: Mo and W: 0.2-3.0% in terms of Mo+0.5W; and
- Third group elements: Ca: 0.001-0.05%, Mg: 0.001-0.05%, La:
0.001-0.05%, and Ce: 0.001-0.05%.

The martensitic stainless steel of this invention has the basic composition, and further satisfies any of the following inequalities (1)-1 to (1)-4, and the following inequality (2) as specified in claims 1 to 8. In the case of the basic composition described above, or a composition further containing the third group element (s): $M = 98 + 47 ⁢ C - 1.1 ⁢ Cr + 1.4 ⁢ Ni - 150 ⁢ Al ≧ 50$

In the case where only the first group element(s), or further the third group element(s) are contained in the composition: $M = 98 + 47 ⁢ C - 1.1 ⁢ Cr + 1.4 ⁢ Ni - 150 ⁢ Al - 200 ⁢ Nb - 50 ⁢ Ti - 200 ⁢ Zr ≧ 50$

In the case where only the second group element(s), or further the third group element(s) are contained in the composition: $M = 98 + 47 ⁢ C - 1.1 ⁢ Cr + 1.4 ⁢ Ni - 150 ⁢ Al - 22 ⁢ \left(Mo+0.5⁢W\right) ≧ 50$

In the case where the first and second group element(s), or further the third group element(s) are contained in the composition: $M = 98 + 47 ⁢ C - 1.1 ⁢ Cr + 1.4 ⁢ Ni - 150 ⁢ Al - 200 ⁢ Nb - 50 ⁢ Ti - 200 ⁢ Zr - 22 ⁢ \left(Mo+0.5⁢W\right) ≧ 50$ $P ≦ 0.046 - 0.0008 HRC$
where the symbols of the elements in the inequalities (1)-1 to (1)-4, and the inequality (2) indicate the contents (% by mass) of the respective elements, and HRC in the inequality (2) indicates the 5 Rockwell C-scale hardness of the steel as quenched. Note that the inequalities (1)-1 to (1)-4 will be collectively referred to as "inequality (1)" in the following description

### Brief Description of the Drawings

FIG. 1 is a diagram showing a relationship among the P (phosphorus) content, hardness as quenched, and corrosion resistance of a martensitic stainless steel;
FIG. 2 is a table showing the chemical compositions of test materials used in examples;
FIG. 3 is another table showing the chemical compositions of test materials used in examples;
FIG. 4 is a table showing the test results of the examples; and
FIG. 5 is another table showing the test results of the examples.

### Best Mode for Carrying out the Invention

A stainless steel of this invention has the properties described previously in (a) to (c), as a combined effect of the previously described basic compositions, and the conditions specified by the inequalities (1) and (2). Among those, the most significant characteristic feature is that the steel of this invention has no risk of cracking, even if subjected to cathodic protection, as welded. Thus, this feature will be described first.

A welding heat affected zone is heated through a weld heat input, and is thereafter rapidly cooled by the chill effect of the base metal. Its heat pattern is substantially the same as that for quenching. Therefore, the inventors thought, on the assumption that the steel would be used as welded, that the phenomena of corrosion and cracking due to cathodic protection observed at the welding heat affected zone could be evaluated in terms of the phenomena observed in a steel as quenched. Hence, specimens of a 13Cr martensitic stainless steel as quenched were prepared and their metallographic structure, corrosion resistance to carbon dioxide, and a tendency toward cracking due to cathodic protection, were investigated. As a result, it was clarified that in order to prevent carbon dioxide corrosion and cracking due to cathodic protection, the following conditions 1 and 2 need to be satisfied at the same time.
1. The rate of martensite of a metallographic structure as quenched needs to be 95% or more.
2. A relationship between the content of P (phosphorus) and hardness (HRC) as quenched of a steel needs to satisfy P ≦ 0.046-0.0008HRC (the previously described inequality (2)).

The fact that the rate of martensite is less than 95% means that the steel has a structure other than martensite, e.g., austenite or ferrite mixed in a large amount, and in this case, cracking tends to occur under cathodic protection. This is due to corrosion being promoted at regions other than the martensitic structure, and thus hydrogen is produced by the corrosion reaction, which in turn increases the amount of hydrogen absorbed into the steel.

A structure which is quenched at a rate of martensite of 95% or more can be obtained by adjusting the chemical composition of the steel. A specific condition for the adjustment of the chemical composition is the previously described inequality (1). That inequality is an empirical formula obtained from the results of a number of tests conducted by the inventors.

FIG. 1 is a diagram showing the results of carbon dioxide corrosion tests and cracking tests under cathodic protection, which will later be described in "Example". The base steel consists of C: 0.01-0.039%, Si: 0.31-0.36%, Mn: 1.09-2.60%, S: 0.003-0.005%, Cr: 11.7-12.2%, Ni: 1.8-2.1%, Al: 0.08-0.11%, and the balance of Fe. Test specimens were prepared from the base steel by varying the P content and the hardness as quenched in varying degrees. Note that the test specimens were obtained by adjusting the chemical compositions so as to become structures whose rate of martensite is 95% or more as quenched (so as to satisfy the previously described inequality (1)), with their hardness varied by adjusting the contents of C and Mn.

The lower part demarcated by the straight line L in FIG. 1 is a region where the steels exhibit excellent corrosion resistance to carbon dioxide and suffer no cracking under cathodic protection. Since the straight line L is expressed as P=0.046-0.0008HRC, the above-described desired region can be expressed as P ≦ 0.046-0.0008HRC (inequality (2)). What is meant by this inequality (2) is that the hardness of a steel as quenched can be comparatively high if the P content is low, while the hardness of a steel as quenched needs to be low if the P content is comparatively high.

The reasons why the basic composition of the steel according to this invention has been determined as above will be described below. Note that the unit "%" herein means "% by mass" unless otherwise specified.

### C:

When the content of C exceeds 0.04%, the hardness of a steel as quenched, whose rate of martensite is 95% or more, becomes too high to suffer cracking under cathodic protection. The lower the C content, the better. Therefore, the C content is set at 0.04% or less. The lower the C content is, the more satisfactory the toughness of the heat affected zone of the steel as welded becomes, therefore, the desirable upper limit of the C content is 0.025%, and the more desirable upper limit is 0.015%. Note that the lower limit is on the order of 0.001% from the viewpoint of manufacturing the steel economically.

### Si:

Silicon is an element necessary to deoxidize steels. When its content exceeds 1.0%, hot workability is degraded. Therefore, its upper limit is set at 1.0%. No deoxidizing effect can be obtained when the Si content is less than 0.01%.

### Mn:

Manganese is also an element necessary as a deoxidizer for steels. When its content exceeds 1.5%, hot workability is degraded, therefore, its upper limit is set at 1.5%. No deoxidizing effect can be obtained when the Mn content is less than 0.1%.

### Cr:

Chromium is an element for improving corrosion resistance to carbon dioxide and no sufficient corrosion resistance to carbon dioxide can be obtained when the Cr content is less than 7%. On the other hand, when the Cr content exceeds 15%, it is difficult to obtain a rate of martensite of 95% or more for steels as quenched, therefore, the Cr content is set between 7 and 15%. Preferably, it is between 9 and 13%.

### Ni:

In order to obtain a rate of martensite of 95% or more as quenched, the Ni content of a steel needs to be in the range of its than 4.0 0.7-less than 4.0, because when the Ni content is less than 0.7%, the formation of ferrite is promoted. Note that excellent properties can be obtained even if the Ni content is within such a low range of 0.7 to less than 4.0%, and thus a possible reduction in the material costs is one of the characteristic features of the steel according to this invention.

### A1:

Similarly to Si, Al is a necessary element as a deoxidizer in the steel making process. When its content is less than 0.001%, no desired deoxidizing effect can be obtained. On the contrary, when its content exceeds 0.20%, nonmetallic inclusions increase and thus the corrosion resistance is degraded. Hence, the Al content was set between 0.001 and 0.20%.

### Cu:

Although not an essential element, Cu has the effect of suppressing the corrosion of steels and reducing the production of hydrogen to thereby prevent cracking under cathodic protection, and thus Cu can be added whenever necessary. However, when its content exceeds 2%, its effect gets saturated. Therefore, even if Cu is added, it is desirable that its content is up to 2%.

### N:

When the content of N exceeds 0.05%, the hardness of the welding heat affected zone of a steel as quenched, becomes so high that the steel is susceptible to cracking under cathodic protection. Therefore, the N content should be kept at 0.05% or lower.

### P:

One of the significant characteristic features of this invention is that the content of P is regulated in relation to the hardness (HRC) of an as-quenched steel. The reasons for such regulation have already been described.

Note that a P content in excess of 0.03% causes the action of promoting sulfide corrosion cracking to appear in hydrogen sulfide environments and thus it is desirable to adjust the chemical composition of a steel, so as to satisfy the previously described inequality (2) with the tolerable upper limit of P set at 0.03%.

### S:

Sulfur is also present as an impurity in steels. Since S impairs hot workability when its content exceeds 0.01%, its upper limit is set at 0.01%. The less, the better. However, the lower limit, permitting economical manufacture, is on the order of 0.0007%.

### First Group Elements (Nb, Ti, Zr):

One or more of Nb, Ti and Zr are added whenever necessary in order to fix C and reduce fluctuations in strength. Content of each of these elements, in an amount of less than 0.005%, is not effective. Content of each in an amount exceeding 0.10% cannot achieve a rate of martensite of 95% or more, and the hardness of a steel as quenched also becomes so high that the risk of cracking, due to cathodic protection, is increased. Note that these elements may be added singly or in combination of two or more.

Since the first group elements are not essential, none of them need be added at all. However, some addition of them in slight amounts, provides the effect of fixing C, so it is desirable to add them, considering the economy, in the range of less than 5 x C (%) Nb, less than 4 x C(%)Ti, and less than 10 x C(%)Zr.

### Second Group Elements (Mo, W):

Molybdenum and tungsten are elements that prevent localized corrosion in carbon dioxide environments, while present with Cr, therefore, for steels used in particularly severe corrosive environments, it is desirable that the steel contains one or both Mo and W in amounts ranging from 0.2 to 3.0% in terms of "Mo+0.5W." No sufficient improvement of localized corrosion resistance is observed with their contents being less than 0.2%, while there is little increase in their effect when the amounts exceed 0.3%.

### Third Group Elements (Ca, Mg, La, Ce):

All of Ca, Mg, La and Ce are effective in improving the hot workability of steels. Therefore, to obtain this effect, one, or two or more of them may be selected and added. However, the above-described effect cannot be obtained when content of any of these elements is less than 0.001%. On the other hand, a content exceeding 0.05% produces coarse oxides, which reduce the corrosion resistance of steels, therefore, when these elements are added, each of the contents should be between 0.001 and 0.05%. Note that Ca and La are particularly preferable among these elements.

The martensitic stainless steel of this invention is used after subjected it to a quenching-tempering heat treatment. This heat treatment may be carried out under ordinary conditions; for example, a water quenching process from the temperature of Ar, point or higher and a subsequent tempering process at 600-670°C, for 5-60 minutes, may be performed. Through such heat treatment, the steel of this invention is given a proof stress of 550MPa or more and an excellent toughness.

When welded, the heat affected zone that comes in contact with the weld metal is brought to a quenched state, and thus it has an extreme hardness. Even in this state, the heat affected zone of the steel, according to this invention, is satisfactory in toughness and corrosion resistance with its rate of martensite being 95% or more, and also has no risk of cracking under cathodic protection. Note that it is, of course, further desirable to subject the steel to a heat treatment (PWHT) for the purpose of softening the heat affected zone, after welding.

Next, the effects of this invention will be described more specifically by way of examples.

### Examples

Steels whose chemical compositions are as shown in FIGS. 2 and 3 were prepared by melting with an ordinary electric furnace and by refining with an argon-oxygen decarburizing furnace (AOD furnace) for desulfurization. The steels were cast into 500-mm-diameter ingots, and billets having 150 mm in diameter were obtained by hot forging the ingots at 1200°C. Seamless steel pipes, having 168 mm in outside diameter and 12 mm in thickness, were manufactured by the Mannesmann pipe making process.

The following test materials were prepared from the above described seamless steel pipes.
(a) Pipes quenched by air cooling or water cooling, after heated for 30 minutes, at 950°C.
(b) Pipes subjected to tempering in which the pipes described in (a) above were heated for 30 minutes at 600°C and thereafter air-cooled.
(c) Welded pipes obtained by peripherally welding the pipes described in (b) above.

The welding of the pipes of (c) was effected in accordance with ASTM 1G by a gas-tungsten arc welding method (GTAW) or a shield metal arc welding method (SMAW), using a welding material made of a 25Cr duplex stainless steel.

The following tests were conducted using the test materials described in (a) to (c) above.

### (A) Measurement of Hardness

Cross-sections perpendicular to their longitudinal direction were cut out of the as-quenched pipes, previously described in (a), and their HRC hardnesses were measured.

### (B) Rate of Martensite

Cross-sections perpendicular to their longitudinal direction were cut out of the as-quenched pipes previously described in (a), and ten views of their microstructure were observed for each of the cross-sections, at a magnification of 100, using an optical microscope to thereby measure the rates of martensite (area rates) and obtain the average.

### (C) Tensile Test

Test specimens having 4.0-mm-diameter and 20-mm-long parallel portion were obtained from the quenched-tempered material previously described in (b). These test specimens were subjected to a tensile test, at ambient temperature, to obtain 0.2% proof stresses.

### (D) Charpy Test

Full-size Charpy test specimens (10 mm x 10 mm x 55 mm, 2 mm V-notch) were cut out of the welding heat affected zones of the as-welded pipes previously described in (c), and were tested at varying temperatures, to obtain the temperatures at which their rate of brittle fracture surface becomes 50%.

### (E) Carbon Dioxide Corrosion Test

Test specimens measured 22 mm (w) x 3 mm (t) x 76 mm (1), which were cut out of the as-welded test material previously described in (c), polished with an emery paper No.600, and thereafter degreased and dried, were used. The test specimens were cut out of locations including the welding heat affected zone and the weld metal.

The above-described test specimens were immersed for 720 hours in a 5%NaCl aqueous solution (the temperature of the solution was 125°C and the flow velocity was 3.5 m/s) in which CO₂ was saturated at a pressure of 30 atm.

Then, if the test specimens suffered localized corrosion or not was visibly observed, and a mass loss (the value obtained by subtracting the weight of each test specimen after the test from the weight of each test specimen before the test) of each test specimen was measured, and the mass loss was converted into a corrosion rate (mm/year).

### (F) Cracking Test under Cathodic Protection

Using test specimens cut out of locations including the welding heat affected zone and the weld metal of the as-welded test material previously described in (c), tests were conducted under the following conditions.
- Testing solution:: Artificial seawater
- Potential:: -1300 mV vs.SCE
- Testing temperature:: 25°C
- Immersion time:: 720 hours
- Applied stress:: 100% of the 0.2% proof stress of the base metal
- Test specimens:: 10 mm (w) x 2mm (t) x 75 mm (1) (for four-point bending test)

The results of the above tests are shown in FIGS. 4 and 5. In these drawings, the marks "O" and "x" indicated in the columns have the following meanings.

In the column for toughness;
- O:: Temperature, wherein the rate of brittle fracture surface is 50%, is -30°C or lower.
- x:: Temperature, wherein the rate of brittle fracture surface is 50%, is higher than -30°C.

In the column for corrosion resistance to carbon dioxide
- O:: Corrosion rate is 0.05 mm/year or less and no localized corrosion observed.
- x:: Corrosion rate exceeds 0.05 mm/year and localized corrosion observed, or localized corrosion observed even if corrosion rate is 0.05 mm/year or less.

In the column for cracking under cathodic protection
- O:: No cracking observed
- x:: Cracking observed

The test Nos. 1 to 44 except those marked "x" shown in FIGS. 2 and 3 are stainless steels according to this invention. The rates of martensite of these steels as-quenched and their values M calculated from the previously described inequality (1) are shown in FIGS. 4 and 5. Further, the allowable upper limits of hardness (HRC) calculated from the previously described inequality (2), i.e., the values of (0.046-P)/0.0008 are also presented in these drawings.

It is apparent from the test results shown in FIGS. 4 and 5, that all the steels exhibited a rate of martensite of 95% or more as quenched, and their 0.2% proof stresses, after subjected to the quenching-tempering treatment, are 550MPa or more. These steels do not suffer cracking under cathodic protection even as welded, and were also excellent in corrosion resistance to carbon dioxide.

The above-described excellent properties are provided by the combined effect of the basic chemical composition being appropriate, the rate of martensite of 95% or more as quenched being achieved by satisfying the previously described inequality (1), and the relationship between the P content and hardness (HRC) satisfying the previously described inequality (2).

Test Nos. 45 to 62 steels of FIG. 3 were prepared as comparative examples. In these steels, Nos. 53 to 55 steels and Nos. 60 to 62 steels, whose chemical compositions are outside the range specified by this invention are, as shown in FIG. 5, inferior in part or in whole in their properties as welded.

Test Nos. 45, 48 to 52 and 56 to 59 steels do not satisfy the condition specified by the previously described inequality (2). That is, their hardnesses after quenching exceed the allowable upper limits calculated from the inequality (2). These steels suffer cracking under cathodic protection. Test Nos. 46 and 47 steels have their M values less than 50 and these steels have low rates of martensite after quenching, and thus poor in toughness, and suffer cracking under cathodic protection.

### Industrial Applicability

The martensitic stainless steel of this invention is a high-strength, high-toughness steel, excellent in corrosion resistance to carbon dioxide, and has no risk of cracking even if used as welded under cathodic protection. This steel is extremely suitable for use as linepipe for transporting crude oil and the like, which contain carbon dioxide, particularly, while subjected to cathodic protection in the sea. Since this steel requires no heat treatment after welded, it can exhibit the economy of a martensitic stainless steel at a satisfactory level, and thus has a significant practical advantage.

## Claims

1. A high-corrosion-resistant martensitic stainless steel, which is used under cathodic protection, **characterized by** consisting, on a mass basis, of: C: not greater than 0.04%, Si: 0.01-1.0%, Mn: 0.1-1.5%, Cr: 7-15%, Ni: 0.7-less than 4.0%, Al: 0.001-0.20%, Cu: 0-2 S : not greater than 0.01%, N: not greater than 0.05%, the balance of Fe and incidental impurities, and further **characterized by** satisfying the following inequalities (1)-1 and (2): $M = 98 + 47 ⁢ C - 1.1 ⁢ Cr + 1.4 ⁢ Ni - 150 ⁢ Al ≧ 50$ $P ≦ 0.046 - 0.0008 HRC$
where the symbols of the elements in the inequalities (1)-1 and (2) indicate the contents (% by mass) of the respective elements, and HRC in the inequality (2) indicates the Rockwell C-scale hardness of the steel as quenched.

2. A high-corrosion-resistant martensitic stainless steel, which is used under cathodic protection, **characterized by** consisting, on a mass basis, of: C: not greater than 0.04%, Si: 0.01-1.0%, Mn: 0.1-1.5%, Cr: 7-15%, Ni: 0.7- less than 4,0 %, Al: 0.001-0.20%, Cu: 0-2, S: not greater than 0.01%, N: not greater than 0.05%, one or more of the following first group elements, the balance of Fe and incidental impurities, and further **characterized by** satisfying the following inegalities (1)-2 and (2):
| | |
|---|---|
| First group elements | Nb: 0,005-0,10 %, Ti: 0,005-0,10 %, |
| | und Zr: 0,005-0,10 % |
$M = 98 + 47 ⁢ C - 1.1 ⁢ Cr + 1.4 ⁢ Ni - 150 ⁢ Al - 200 ⁢ Nb - 50 ⁢ Ti - 200 ⁢ Zr ≧ 50$ $P ≦ 0.046 - 0.0008 HRC$
where the symbols of the elements in the inequalities (1)-2 and (2) indicate the contents (% by mass) of the respective elements, and HRC in the inequality (2) indicates the Rockwell C-scale hardness of the steel as quenched.

3. A high-corrosion-resistant martensitic stainless steel, which is used under cathodic protection, **characterized by** consisting, on a mass basis, of: C: not greater than 0.04%, Si: 0.01-1.0%, Mn: 0.1-1.5%, Cr: 7-15%, Ni: 0.7-less than 4.0%, Al: 0.001-0.20%, Cu: 0-2, S: not greater than 0.01%, N: not greater than 0.05%, one or more of the following second group elements, the balance of Fe and incidental impurities, and further **characterized by** satisfying the following inequalities (1)-3 and (2):
| | |
|---|---|
| Second group elements | Mo and W: 0.2-3.0% in terms of |
| | Mo+0.5W |
$M = 98 + 47 ⁢ C - 1.1 ⁢ Cr + 1.4 ⁢ Ni - 150 ⁢ Al - 22 ⁢ \left(Mo+0.5⁢W\right) ≧ 50$ $P ≦ 0.046 - 0.0008 HRC$
where the symbols of the elements in the inequalities (1)-3 and (2) indicate the contents (% by mass) of the respective elements, and HRC in the inequality (2) indicates the Rockwell C-scale hardness of the steel as quenched.

4. A high-corrosion-resistant martensitic stainless steel, which is used under cathodic protection, **characterized by** consisting, on a mass basis, of: C: not greater than 0.04%, Si: 0.01-1.0%, Mn: 0.1-1.5%, Cr: 7-15%, Ni: 0.7-less than 4.0%, Al: 0.001-0.20%, Cu: 0-2, S: not greater than 0.01%, N: not greater than 0.05%, one or more of the following third group elements, the balance of Fe and incidental impurities, and further **characterized by** satisfying the following inequalities (1)-.1 and (2):
| | |
|---|---|
| Third group elements | Ca: 0.001-0.05%, Mg: 0.001-0.05%, |
| | La: 0.001-0.05%, and Ce: 0.001-0.05% |
$M = 98 + 47 ⁢ C - 1.1 ⁢ Cr + 1.4 ⁢ Ni - 150 ⁢ Al ≧ 50$ $P ≦ 0.046 - 0.0008 ⁢ HRC$ where the symbols of the elements in the inequalities (1)-1 and (2) indicate the contents (% by mass) of the respective elements, and HRC in the inequality (2) indicates the Rockwell C-scale hardness of the steel as quenched.

5. A high-corrosion-resistant martensitic stainless steel, which is used under cathodic protection, **characterized by** consisting, on a mass basis, of: C: not greater than 0.04%, Si: 0.01-1.0%, Mn: 0.1-1.5%, Cr: 7-15%, Ni: 0.7- less than 4.0%, Al: 0.001-0.20%, Cu: 0-2, S: not greater than 0.01%, N: not greater than 0.05%, one or more of the following first group elements, one or more of the following second group elements, the balance of Fe and incidental impurities, and further **characterized by** satisfying the following inequalities (1)-4 and (2):
| | |
|---|---|
| First group elements | Nb: 0.005-0-10%, Ti: 0.005.-0.10%, |
| | and Zr: 0.005-0.10% |
| Second group elements | Mo and W; 0.2-3.0% in terms of |
| | Mo+0.5W |
$M = 98 + 47 ⁢ C - 1.1 ⁢ Cr + 1.4 ⁢ Ni - 150 ⁢ Al - 200 ⁢ Nb - 50 ⁢ Ti - 200 ⁢ Zr - 22 ⁢ \left(Mo+0.5⁢W\right) ≧ 50$ $P ≦ 0.046 - 0.0008 HRC$
where the symbols of the elements in the inequalities (1) -4 and (2) indicate the contents (% by mass) of the respective elements, and HRC in the inequality (2) indicates the Rockwell C-scale hardness of the steel as quenched.

6. A high-corrosion-resistant martensitic stainless steel, which is used under cathodic protection, **characterized by** consisting, on a mass basis, of: C: not greater than 0.04%, si: 0.01-1.0%, Mn: 0.1-1.5%, Cr: 7-15%, Ni: 0.7- less than 4.0%, Al: 0.001-0.20%, Cu: 0-2, S: not greater than 0.01%, N: not greater than 0.05%, one or more of the following first group elements, one or more of the following third group elements, the balance of Fe and incidental impurities, and further by satisfying the following inequalities -2 and (2):
| | |
|---|---|
| First group elements | Nb: 0.005-0-10%, Ti: 0.005.-0.10%, |
| | and Zr: 0.005-0.10% |
| Third group elements | Ca: 0.001-0.05%, Mg: 0.001-0.05%, |
| | La: 0.001-0.05%, and Ce: 0.001-0.05% |
${M = 98 + 47 ⁢ C - 1.1 ⁢ Cr + 1.4 ⁢ Ni - 150 ⁢ Al - 200 ⁢ Nb - 50 ⁢ Ti - 200 ⁢ Zr ≧ 50}_{̲}$ $P ≦ 0.046 - 0.0008 HRC$
where the symbols of the elements in the inequalities (1) -2 and (2) indicate the contents (% by mass) of the respective elements, and HRC in the inequality (2) indicates the Rockwell C-scale hardness of the steel as quenched.

7. A high-corrosion-resistant martensitic stainless steel, which is used under cathodic protection, **characterized by** consisting , on a mass basis, of: C: not greater than 0.04%, Si: 0.01-1.0%, Mn: 0.1-1.5%, Cr: 7-15%, Ni: 0.7-less than 4.0%, Al: 0.001-0.20%, Cu: 0-2, S: not greater than 0.01%, N: not greater than 0.05%, one of more of the following second group elements, one or more of the following third group elements, the balance of Fe and incidental impurities, and further **characterized by** satisfying the following inequalities (1)-3 and (2):
| | |
|---|---|
| Second group elements | Mo and W: 0.2-3.0% in terms of |
| | Mo+0.5w |
| Third group elements | Ca: 0.001-0.05%, Mg: 0.001-0.05%, |
| | La: 0.001-0.05%, and Ce: 0.001-0.05% |
$M = 98 + 47 ⁢ C - 1.1 ⁢ Cr + 1.4 ⁢ Ni - 150 ⁢ Al - 22 ⁢ \left(Mo+0.5⁢W\right) ≧ 50$ $P ≦ 0.046 - 0.0008 HRC$
where the symbols of the elements in the inequalities (1)-3 and (2) indicate the contents (% by mass) of the respective elements, and HRC in the inequality (2) indicates the Rockwell c-scale hardness of the steel as quenched.

8. A high-corrosion-resistant martensitic stainless steel, which is used under cathodic protection, **characterized by** consisting, on a mass basis, of: C: not greater than 0.04%, Si: 0.01-1.0%, Mn: 0.1-1.5%, Cr: 7-15%, Ni : 0.7-less than 4.0%, Al: 0.001-0.20%, Cu: 0-2, S: not greater than 0.01%, N: not greater than 0.05%, one or more of the following first group elements, one or more of the following second group elements, one or more of the following third group elements, the balance of Fe and incidental impurities, and further **characterized by** satisfying the following inequalities (1)-4 and (2):
| | |
|---|---|
| First group elements | Nab: 0.005-0-10%, Ti**:** 0.005-0.10%, |
| | and zr: 0.005-0.10% |
| Second group elements | Mo and W: 0.2-3.0% in terms of Mo+0.5W |
| Third group elements | Ca: 0.001-0.05%, Mg: 0.001-0.05% |
| | La: 0.001-0.05%, and Ce: 0.001-0.05% |
$M = 98 + 47 ⁢ C - 1.1 ⁢ Cr + 1.4 ⁢ Ni - 150 ⁢ Al - 200 ⁢ Nb - 50 ⁢ Ti - 200 ⁢ Zr - 22 ⁢ \left(Mo+0.5⁢W\right) ≧ 50$ $P ≦ 0.046 - 0.0008 HRC$
where the symbols of the elements in the inequalities (1)-4 and (2) indicate the contents (% by mass) of the respective elements, and HRC in the inequality (2) indicates the Rockwell C-scale hardness of the steel as quenched.

9. A steel pipe for use in seawater while subjected to cathodic protection, which is made of a steel according to any of claims 1 to 8.

## Revendications

1. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %, Ni : de 0,7 à moins de 4,0 %, Al : de 0,001 à 0,20 %, Cu : de 0 à 2 %, S : pas plus de 0,01 %, N : pas plus de 0,05 %, le complément en Fe et impuretés éventuelles et
**caractérisé, en outre, en ce qu'**il satisfait les inégalités (1)-1 et (2) suivantes : $M = 98 + 47 ⁢ C - 1 , 1 ⁢ Cr + 1 , 4 ⁢ Ni - 150 ⁢ Al ≧ 50$$P ≦ 0 , 046 - 0 , 0008 HRC$
où les symboles des éléments dans les inégalités (1)-1 et (2) indiquent les teneurs (% en poids) des éléments respectifs, et HRC dans l'inégalité (2) indique l'échelle C de dureté Rockwell de l'acier à l'état trempé.

2. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %, Ni : de 0,7 à moins de 4,0 %, Al : de 0,001 à 0,20 %, Cu : de 0 à 2 %, S : pas plus de 0,01 %, N : pas plus de 0,05 %, un ou plusieurs des éléments du premier groupe suivant, le complément en Fe et impuretés éventuelles et **caractérisé, en outre, en ce qu'**il satisfait les inégalités (1)-2 et (2) suivantes :
éléments du premier groupe : Nb : de 0,005 à 0,10 %, Ti : de 0,005 à 0,10 %, et Zr : de 0,005 à 0,10 % $M = 98 + 47 ⁢ C - 1 , 1 ⁢ Cr + 1 , 4 ⁢ Ni - 150 ⁢ Al - 200 ⁢ Nb - 50 ⁢ Ti - 200 ⁢ Zr \geq 50$ $P ≦ 0 , 046 - 0 , 0008 HRC$
où les symboles des éléments dans les inégalités (1)-2 et (2) indiquent les teneurs (% en poids) des éléments respectifs, et HRC dans l'inégalité (2) indique l'échelle C de dureté Rockwell de l'acier à l'état trempé.

3. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %, Ni : de 0,7 à moins de 4,0 %, Al : de 0,001 à 0,20 %, Cu : de 0 à 2 %, S : pas plus de 0,01 %, N : pas plus de 0,05 °lo, un ou plusieurs des éléments du deuxième groupe suivant, le complément en Fe et impuretés éventuelles et **caractérisé, en outre, en ce qu'**il satisfait les inégalités (1)-3 et (2) suivantes :
éléments du deuxième groupe : Mo et W : de 0,2 à 3,0 % pour le total de Mo + 0,5 W
$M = 98 + 47 ⁢ C - 1 , 1 ⁢ Cr + 1 , 4 ⁢ Ni - 150 ⁢ Al - 22 ⁢ \left(Mo+0,5⁢W\right) \geq 50$ $P \leq 0 , 046 - 0 , 0008 HRC$
où les symboles des éléments dans les inégalités (1)-3 et (2) indiquent les teneurs (% en poids) des éléments respectifs, et HRC dans l'inégalité (2) indique l'échelle C de dureté Rockwell de l'acier à l'état trempé.

4. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %, Ni : de 0,7 à moins de 4,0 %, Al : de 0,001 à 0,20 %, Cu : de 0 à 2 %, S : pas plus de 0,01 %, N : pas plus de 0,05 %, un ou plusieurs des éléments du troisième groupe suivant, le complément en Fe et impuretés éventuelles et **caractérisé, en outre, en ce qu'**il satisfait les inégalités (1)-1 et (2) suivantes :
éléments du troisième groupe : Ca : de 0,01 à 0,05 %, Mg : de 0,001 à 0,5 %, La : de 0,001 à 0,05 % et Ce : de 0,001 à 0,05 %
$M = 98 + 47 ⁢ C - 1 , 1 ⁢ Cr + 1 , 4 ⁢ Ni - 150 ⁢ Al \geq 50$ $P \leq 0 , 046 - 0 , 0008 HRC$
où les symboles des éléments dans les inégalités (1)-1 et (2) indiquent les teneurs (% en poids) des éléments respectifs, et HRC dans l'inégalité (2) indique l'échelle C de dureté Rockwell de l'acier à l'état trempé.

5. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %; Ni : de 0,7 à moins de 4,0 %, Al : de 0,001 à 0,20 %, Cu : de 0 à 2 %, S : pas plus de 0,01 %, N : pas plus de 0,05 %, un ou plusieurs des éléments du premier groupe suivant, un ou plusieurs des éléments du deuxième groupe suivant, le complément en Fe et impuretés éventuelles et **caractérisé, en outre, en ce qu'**il satisfait les inégalités (1)-4 et (2) suivantes :
éléments du premier groupe : Nb : de 0,005 à 0,10 %, Ti : de 0,005 à 0,10 %, et Zr : de 0,005 à 0,10 %
éléments du deuxième groupe : Mo et W : de 0,2 à 3,0 % pour le total de Mo + 0,5 W $M = 98 + 47 ⁢ C - 1 , 1 ⁢ Cr + 1 , 4 ⁢ Ni - 150 ⁢ Al - 200 ⁢ Nb - 50 ⁢ Ti - 200 ⁢ Zr - 22 ⁢ \left(Mo+0,5⁢W\right) \geq 50$ $P \leq 0 , 046 - 0 , 0008 HRC$
où les symboles des éléments dans les inégalités (1)-4 et (2) indiquent les teneurs (% en poids) des éléments respectifs, et HRC dans l'inégalité (2) indique l'échelle C de dureté Rockwell de l'acier à l'état trempé.

6. Acier inoxydable martensitique à haute résistance à la corrosion, qui est utilisé sous protection cathodique, **caractérisé en ce qu'**il consiste, sur une base en poids, en : C: pas plus de 0,04 %, Si : de 0,01 à 1,0 %, Mn : de 0,1 à 1,5 %, Cr : de 7 à 15%, Ni : de 0,7 à moins de 4,0 %, Al: de 0,001 à 0,20 %, Cu : de 0 à 2 %, S : pas plus de 0,01 %, N : pas plus de 0,05 %, un ou plusieurs des éléments du premier groupe suivant, un ou plusieurs des éléments du troisième groupe suivant, le complément en Fe et impuretés éventuelles et **caractérisé, en outre, en ce qu'**il satisfait les inégalités (1)-2 et (2) suivantes :
éléments du premier groupe : Nb : de 0,005 à 0,10 %, Ti : de 0,005 à 0,10 %, et Zr: de 0,005 à 0,10 %
éléments du troisième groupe : Ca : de 0,01 à 0,05 %, Mg : de 0,001 à 0,5 %, La : de 0,001 à 0,05 % et Ce : de 0,001 à 0,05 %
$M = 98 + 47 ⁢ C - 1 , 1 ⁢ Cr + 1 , 4 ⁢ Ni - 150 ⁢ Al - 200 ⁢ Nb - 50 ⁢ Ti - 200 ⁢ Zr \geq 50$ $P \leq 0 , 046 - 0 , 0008 HRC$
où les symboles des éléments dans les inégalités (1)-2 et (2) indiquent les teneurs (% en poids) des éléments respectifs, et HRC dans l'inégalité (2) indique l'échelle C de dureté Rockwell de l'acier à l'état trempé.

7. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %, Ni : de 0,7 à moins de 4,0 %, Al : de 0,001 à 0,20 %, Cu : de 0 à 2 %, S : pas plus de 0,01 %, N : pas plus de 0,05 %, un ou plusieurs des éléments du deuxième groupe suivant, un ou plusieurs des éléments du troisième groupe suivant, le complément en Fe et impuretés éventuelles et **caractérisé, en outre, en ce qu'**il satisfait les inégalités (1)-3 et (2) suivantes :
éléments du deuxième groupe : Mo et W : de 0,2 à 3,0 % pour le total de Mo + 0,5 W
éléments du troisième groupe : Ca : de 0,01 à 0,05 %, Mg : de 0,001 à 0,5 %, La : de 0,001 à 0,05 % et Ce : de 0,001 à 0,05 %
$M = 98 + 47 ⁢ C - 1 , 1 ⁢ Cr + 1 , 4 ⁢ Ni - 150 ⁢ Al - 22 ⁢ \left(Mo+0,5⁢W\right) \geq 50$ $P \leq 0 , 046 - 0 , 0008 HRC$
où les symboles des éléments dans les inégalités (1)-3 et (2) indiquent les teneurs (% en poids) des éléments respectifs, et HRC dans l'inégalité (2) indique l'échelle C de dureté Rockwell de l'acier à l'état trempé.

8. Acier inoxydable martensitique à haute résistance à la corrosion, qui est utilisé sous protection cathodique, **caractérisé en ce qu'**il consiste, sur une base en poids, en : C : pas plus de 0,04 %, Si : de 0,01 à 1,0 %, Mn : de 0,1 à 1,5 %, Cr : de 7 à 15 %, Ni : de 0,7 à moins de 4,0 %, Al : de 0,001 à 0,20 %, Cu : de 0 à 2 %, S : pas plus de 0,01 %, N : pas plus de 0,05 %, un ou plusieurs des éléments du premier groupe suivant, un ou plusieurs des éléments du deuxième groupe suivant, un ou plusieurs des éléments du troisième groupe suivant, le complément en Fe et impuretés éventuelles et **caractérisé, en outre, en ce qu'**il satisfait les inégalités (1)-4 et (2) suivantes :
éléments du premier groupe : Nb : de 0,005 à 0,10 %, Ti : de 0,005 à 0,10 %, et Zr: de 0,005 à 0,10 %
éléments du deuxième groupe : Mo et W : de 0,2 à 3,0 % pour le total de Mo + 0,5 W
éléments du troisième groupe : Ca : de 0,01 à 0,05 %, Mg : de 0,001 à 0,5 %, La : de 0,001 à 0,05 % et Ce : de 0,001 à 0,05 %
$M = 98 + 4 ⁢ C - 1 , 1 ⁢ Cr + 1 , 4 ⁢ Ni - 150 ⁢ Al - 200 ⁢ Nb - 50 ⁢ Ti - 200 ⁢ Zr - 22 ⁢ \left(Mo+0,5⁢W\right) \geq 50$ $P \leq 0 , 046 - 0 , 0008 HRC$
où les symboles des éléments dans les inégalités (1)-4 et (2) indiquent les teneurs (% en poids) des éléments respectifs, et HRC dans l'inégalité (2) indique l'échelle C de dureté Rockwell de l'acier à l'état trempé.

9. Tuyauterie en acier à utiliser dans l'eau de mer, après avoir été soumise à une protection cathodique, qui est réalisée en un acier selon l'une quelconque des revendications 1 à 8.

## Patentansprüche

1. Hochkorrosionsbeständiger, martensitischer, rostfreier Stahl, der unter Kathodenschutz verwendet wird, ***dadurch gekennzeichnet,* dass** er auf einer Massenbasis besteht aus: C: nicht mehr als 0,04 %, Si: 0.01-1,0 %, Mn: 0,1-1,5 %, Cr: 7-15 %; Ni: 0,7- weniger als 4,0 %, Al: 0,001-0,20 %, Cu: 0-2, S: nicht mehr als 0,01 %, N: nicht mehr als 0,05 %, dem Rest Fe und zufälligen Verunreinigungen, und der ferner ***dadurch gekennzeichnet* ist, dass** er die folgenden Ungleichungen (1)-1 und (2) erfüllt: $M = 98 + 47 ⁢ C - 1 , 1 ⁢ Cr + 1 , 4 ⁢ Ni - 150 ⁢ Al \geq 50$ $P \leq 0 , 046 - 0 , 0008 ⁢ HRC$
wobei die Symbole der Elemente in den Ungleichungen (1)-1 und (2) die Gehalte (in Masse-%) der jeweiligen Elemente anzeigen und HRC in der Ungleichung (2) die Rockwellhärte der C-Kennung von vergütetem Stahl anzeigt.

2. Hochkorrosionsbeständiger, martensitischer, rostfreier Stahl, der unter Kathodenschutz verwendet wird, ***dadurch gekennzeichnet,* dass** er auf einer Massenbasis besteht aus: C: nicht mehr als 0,04 %, Si: 0,01-1,0 %, Mn: 0,1-1,5 %, Cr: 7-15 %, Ni: 0,7- weniger als 4,0 %, Al: 0,001-0,20 %, Cu: 0-2, S: nicht mehr als 0,01 %, N: nicht mehr als 0,05 %, einem oder mehreren der folgenden Elemente der ersten Gruppe, dem Rest Fe und zufälligen Verunreinigungen, und der ferner ***dadurch gekennzeichnet* ist, dass** er die folgenden Ungleichungen (1)-2 und (2) erfüllt:
| | |
|---|---|
| Elemente der ersten Gruppe | Nb: 0,005-0,10 %, Ti: 0,005-0,10 %, |
| | und Zr: 0,005-0,10 % |
$M = 98 + 47 ⁢ C - 1 , 4 ⁢ Ni - 150 ⁢ Al - 200 ⁢ Nb - 50 ⁢ Ti - 200 ⁢ Zr \geq 50$ $P \leq 0 , 046 - 0 , 0008 ⁢ HRC$
wobei die Symbole für die Elemente in den Ungleichungen (1)-2 und (2) die Gehalte (in Masse-%) der jeweiligen Elemente angeben und HRC in der Ungleichung (2) die Rockwellhärte der C-Kennung von vergütetem Stahl anzeigt.

3. Hochkorrosionsbeständiger, martensitischer, rostfreier Stahl, der unter Kathodenschutz verwendet wird, ***dadurch gekennzeichnet* dass** er auf einer Massenbasis besteht aus: C: nicht mehr als 0,04 %, Si: 0,01-1,0 %, Mn: 0,1-1,5 %, Cr: 7-15 %, Ni: 0,7- weniger als 4,0 %, Al**:** 0,001-0,20 %, Cu: 0-2, S: nicht mehr als 0,01 %, N: nicht mehr als 0,05 %, einem oder mehreren der folgenden Elemente der zweiten Gruppe, dem Rest Fe und zufälligen Verunreinigungen, und der ferner ***dadurch gekennzeichnet* ist, dass** er die folgenden Ungleichungen (1)-3 und (2) erfüllt:
| | |
|---|---|
| Elemente der zweiten Gruppe | Mo und W: 0,2-3,0 % in Termen von Mo+0,5W |
$M = 98 + 47 ⁢ C - 1 , 1 ⁢ Cr + 1 , 4 ⁢ Ni - 150 ⁢ Al - 22 ⁢ \left(Mo+0,5⁢W\right) \geq 50$ $P \leq 0 , 046 - 0 , 0008 ⁢ HRC$
wobei die Symbole der Elemente den Ungleichungen (1)-3 und (2) die Gehalte (in Masse-%) der jeweiligen Elemente anzeigen, und HRC in der Ungleichung (2) die Rockwellhärte der C-Kennung von vergütetem Stahl anzeigt.

4. Hochkorrosionsbeständiger martensitischer, rostfreier Stahl, der unter Kathodenschutz verwendet wird, ***dadurch gekennzeichnet,* dass** er auf einer Massebasis besteht aus: C: nicht mehr als 0,04 %, Si: 0,01-1,0 %, Mn: 0,1-1,5 %, Cr: 7-15 %, Ni: 0,7- weniger als 4,0 %, Al: 0,001-0,20 %, Cu: 0-2, S: nicht mehr als 0,01 %, N: nicht mehr als 0,05 %, ein oder mehrere der folgenden Elemente der dritten Gruppe, dem Rest Fe und zufälligen Verunreinigungen, und der ferner ***dadurch gekennzeichnet* ist, dass** er die folgenden Ungleichungen (1)-1 und (2) erfüllt:
| | |
|---|---|
| Elemente der dritten Gruppe | Ca: 0,001-0,05 %, Mg: 0,001-0,05 %, |
| | La: 0,001-0,05 %, und Ce: 0,001-0,05 % |
$M = 98 + 47 ⁢ C - 1 , 1 ⁢ Cr + 1 , 4 ⁢ Ni - 150 ⁢ Al \geq 50$ $P \leq 0 , 046 - 0 , 0008 ⁢ HRC$
wobei die Symbole der Elemente in den Ungleichungen (1)-1 und (2) die Gehalte (in Masse-%) der jeweiligen Elemente angeben und HRC in der Ungleichung (2) die Rockwellhärte der C-Kennung von vergütetem Stahl anzeigt.

5. Hochkorrosionsbeständiger, martensitischer, rostfreier Stahl, der unter Kathodenschutz verwendet wird, ***dadurch gekennzeichnet,* dass** er auf einer Massenbasis besteht aus: C: nicht mehr als 0,04 %, Si: 0,01 - 1,0 %, Mn: 0,1-1,5 %, Cr: 7-15 %, Ni: 0,7- weniger als 4,0 %, Al: 0,001-0,20 %, Cu: 0-2, S: nicht mehr als 0,01 %, N: nicht mehr als 0,05 %, ein oder mehrere der folgenden Elemente der ersten Gruppe, ein oder mehrere der folgenden Elemente der zweiten Gruppe, den Rest Fe und zufälligen Verunreinigungen, und der ferner ***dadurch gekennzeichnet* ist, dass** er die folgenden Ungleichungen (1)-4 und (2) erfüllt:
| | |
|---|---|
| Elemente der ersten Gruppe | Nb: 0,005-0,10 %, Ti: 0,005-0,10 %, |
| | und Zr: 0,005-0,10 % |
| Elemente der zweiten Gruppe | Mo und W: 0,2-3,0 % in Termen von Mo+0,5 W |
$M = 98 + 47 ⁢ C - 1 , 1 ⁢ Cr + 1 , 4 ⁢ Ni - 150 ⁢ Al - 200 ⁢ Nb - 50 ⁢ Ti - 200 ⁢ Zr - 22 ⁢ \left(Mo+0,5⁢W\right) \geq 50$ $P \leq 0 , 046 - 0 , 0008 ⁢ HRC$
wobei die Symbole der Elemente in den Ungleichungen (1)-4 und (2) die Gehalte (in Masse-%) der jeweiligen Elemente anzeigen und HRC in der Ungleichung (2) die Rockwellhärte der C-Kennung von vergütetem Stahl anzeigt.

6. Hochkorrosionsbeständiger, martensitischer, rostfreier Stahl, der unter Kathodenschutz verwendet wird, ***dadurch gekennzeichnet,* dass** er auf einer Massebasis besteht aus: C: nicht mehr als 0,04 %, Si: 0,01-1,0 %, Mn: 0,1-1,5 %, Cr: 7-15 %, Ni: 0,7- weniger als 4,0 %, Al: 0,001-0,20 %, Cu: 0-2, S: nicht mehr als 0,01 %, N: nicht mehr als 0,05 %, ein oder mehrere der folgenden Elemente der ersten Gruppe, ein oder mehrere der folgenden Elemente der dritten Gruppe, dem Rest Fe und zufälligen Verunreinigungen und der ferner die folgenden Ungleichungen (1)-2 und (2) erfüllt:
| | |
|---|---|
| Elemente der ersten Gruppe | Nb: 0,005-0,10 %, Ti: 0,005-0,10 % |
| | und Zr: 0,005-0,10 % |
| Elemente der dritten Gruppe | Ca: 0,001-0,05 %, Mg: 0,001-0,05 %, |
| | La: 0,001-0,05 % und Ce: 0,001-0,05 % |
$M = 98 + 47 ⁢ C - 1 , 1 ⁢ Cr + 1 , 4 ⁢ Ni - 150 ⁢ Al - 200 ⁢ Nb - 50 ⁢ Ti - 200 ⁢ Zr \geq 50$ $P \leq 0 , 046 - 0 , 0008 ⁢ HRC$
wobei die Symbole der Elemente in den Ungleichungen (1)-2 und (2) die Gehalte (in Masse-%) der jeweiligen Elemente angeben und HRC in der Ungleichung (2) die Rockwellhärte der C-Kennung von vergütetem Stahl angibt.

7. Hochkonosionsbeständiger, martensitischer, rostfreier Stahl, der unter Kathodenschutz verwendet wird, ***dadurch gekennzeichnet,* dass** er auf einer Massebasis besteht aus: C: nicht mehr als 0,04 %, Si: 0,01-1,0 %, Mn: 0,1-0,5 %, Cr: 7-15 %, Ni: 0,7- weniger als 4,0 %, Al: 0,001-0,20 %, Cu: 0-2, Si: nicht mehr als 0,01 %, N: nicht mehr als 0,05 %, ein oder mehrere der folgenden Elemente der zweiten Gruppe ein oder mehrere der folgenden Elemente der dritten Gruppe, dem Rest Fe und zufälligen Verunreinigungen und der ferner ***dadurch gekennzeichnet* ist, dass** er die folgenden Ungleichungen (1)-3 und (2) erfüllt:
| | |
|---|---|
| Elemente der zweiten Gruppe | Mo und W: 0,2 -3,0 % in Termen von Mo+0,5W |
| Elemente der dritten Gruppe | Ca: 0,001-0,05 %, Mg: 0,001-0,05 %, |
| | La: 0,001-0,05 % und Ce: 0,001-0,05 % |
$M = 98 + 47 ⁢ C - 1 , 1 ⁢ Cr + 1 , 4 ⁢ Ni - 150 ⁢ Al - 22 ⁢ \left(Mo+0,5⁢W\right) \geq 50$ $P \leq 0 , 046 - 0 , 0008 ⁢ HRC$
wobei die Symbole der Elemente der Ungleichungen (1)-3 und (2) die Gehalte (in Masse-%) der jeweiligen Elemente angeben und HRC in der Ungleichung (2) die Rockwellhärte der C-Kennung von vergütetem Stahl angibt.

8. Hochkorrosionsbeständiger, martensitischer, rostfreier Stahl, der unter Kathodenschutz verwendet wird, ***dadurch gekennzeichnet,* dass** er auf einer Massebasis besteht aus: C: nicht mehr als 0,04 %, Si: 0,01-1,0 %, Mn: 0,1-1,5 %, Cr: 7-15 %, Ni: 0,7- weniger als 4,0 %, Al: 0,001-0,20 %, Cu: 0-2, S: nicht mehr als 0,01 %, N: nicht mehr als 0,05 %, ein oder mehrere der folgenden Elemente der ersten Gruppe, ein oder mehrere der folgenden Elemente der zweiten Gruppe, ein oder mehrere der folgenden Elemente der dritten Gruppe, dem Rest Fe und zufälligen Verunreinigungen und der ferner ***dadurch gekennzeichnet* ist, dass** er die folgenden Ungleichungen (1)-4 und (2) erfüllt:
| | |
|---|---|
| Elemente der ersten Gruppe | Nb: 0,005-0,10 %, Ti: 0,005-0,10 % |
| | und Zr: 0,005-0,10 % |
| Elemente der zweiten Gruppe | Mo und W: 0,2-3,0 % in Termen von Mo+0,5W |
| Elemente der dritten Gruppe | Ca: 0,001-0,05 %, Mg: 0,001-0,05 %, |
| | La: 0,001-0,05 % und Ce: 0,041-0,05 % |
$M = 98 + 47 ⁢ C - 1 , 1 ⁢ Cr + 1 , 4 ⁢ Ni - 150 ⁢ Al - 22 ⁢ \left(Mo+0,5⁢W\right) \geq 50$ $P \leq 0 , 046 - 0 , 0008 ⁢ HRC$
wobei die Symbole der Elemente in den Ungleichungen (1)-4 und (2) die Gehalte (in Masse-%) der jeweiligen Elemente angeben und HRC in der Ungleichung (2) die Rockwellhärte der C-Kennung von vergütetem Stahl angibt.

9. Stahlrohr zur Verwendung in Meerwasser bei Aussetzen einem Kathodenschutz, das aus einem Stahl gemäß einem der Ansprüche 1 bis 8 besteht.
